

## UNITED STATES PATENT OFFICE

FRANK S. CARLILE, OF ABINGTON, PENNSYLVANIA

## METHOD OF PREPARING METALLIC MOLDS FOR CASTING METAL

No Drawing.

Application filed August 2, 1930. Serial No. 472,768.

This invention relates to the art of casting metal and is particularly directed to the preparation of metallic molds for casting metal. Although the invention may be generally applied, I have found it of specific value in the production of soft metal castings such for instance as storage battery plates.

It has been the practice to prepare the molds for receiving the molten metal by dusting them with talcum powder or the like or smoking them to form a coating of finely divided carbon, for the purposes of preventing the solidified casting from sticking to the mold, thermally insulating the molten metal to secure proper flowing into the corners and interstices of the mold and allowing the escape of air while the metal is flowing.

The objects of this invention are to provide an improved method of preparing this type of molds for casting, to prevent the solidified cast from adhering to the mold, to secure sharp castings, to vent the mold, to lower the casting temperature, to increase the life of a prepared mold, to facilitate re-preparing a mold, to overcome the defects of prior practice and to generally improve the art of casting metal in metal molds.

I have discovered that if a mold is covered with a coating of fine blisters a surface is produced which materially facilitates the production of desirable castings. I have experimented with applying a varnish froth, of applying various forms of varnish and then heating the mold to form the blisters, of applying varnishes admixed with pre-formed blistered substances, but I find that the best way to produce my desired result is to apply a varnish like material while the mold is maintained at a temperature sufficiently high to cause the varnish to blister as it dries.

Although a number of substances may be used as the said varnish like material, such as nonaqueous solutions of resins, gums, nitrocellulose, pitch or tar, or aqueous solutions of gelatin, casein, albumen, gluten and the like, I have found that a varnish made by admixing evaporated cellulose pulp

waste liquor and water possesses advantages over the other substances which have come within the range of my experiments.

The cellulose pulp waste liquor may be evaporated to dryness and often appears on the market in the form of flour which form I prefer to employ although it should be understood that the degree of evaporation is immaterial so long as the concentration of the dry material in my finished varnish remains the same. Although the amount of water used to form my varnish may be varied over a wide range, I have concluded that the best admixture for my purpose is made by dissolving one pound of the evaporated cellulose pulp waste liquor in the form of flour in nine pounds of water.

To carry out my invention, I heat the mold which is usually of steel, although it may be made of brass or other suitable metal, to a temperature sufficiently high to cause the applied varnish to blister. When the cellulose pulp waste liquor varnish is used the temperature should be 450° F. more or less. I then apply my varnish.

This may be accomplished by dipping, brushing, flow-coating or spraying. I have found that superior results are obtained by spraying. I have found that about one gallon of varnish will cover about 200 square feet of mold surface when a coating of the proper thickness is applied. As soon as the varnish touches the heated surface it at once forms minute blisters.

The mold may now be used for casting, however, I have found that better results are obtained by first breaking many of the blisters before using the mold. This may be accomplished in any manner but I have found that simply lightly brushing the surface accomplishes the result.

It is evident from my description that my process enables me to produce a mold which differs from previous molds in that it has a nonmetallic casting surface of minute blisters or of broken blisters depending on whether or not the final step in my process has been performed.

When my processed mold is used for cast-

100

ing, I have found that the metal may be poured at a lower temperature than heretofore due to the thermal insulation afforded by my coating in preventing the metal from quickly chilling. I have also found, as the heat is better retained by the poured metal, I am not obliged to maintain the mold at so high a temperature by externally applied heat as heretofore and thus the cost of heating is reduced. Owing to this retention of heat, the metal stays fluid longer and thus is allowed sufficient time to enter sharp corners and fine interstices which results in sharp accurate castings. This effect is augmented by the property of my coating in allowing the entrapped air to escape to the vents of the mold. Heretofore much trouble has been encountered by coatings plugging up the said vents but the use of my coating does not produce this condition and thus this trouble is overcome. It has been the custom to coat a mold after each cast but this is not necessary where my coating is employed as I have found one treatment sufficient for making two hundred or more castings. When the time comes however, for recoating the molds, all that is required is to wipe off my coating with water whereupon, due to its solubility in water, it is entirely removed, leaving a surface ready for re-treating.

Although my molds produce very sharp castings, I have noted that the solidified castings do not adhere and are therefore very easily removed, thus saving much time and trouble. This advantage coupled with the lasting properties of my coating and the ease and speed of its application enables molds to be operated by hand or machine at high speed and thus further enable the making of castings at lower cost.

Having thus described my invention, I claim:

1. The method of preparing metallic molds for casting metal consisting in applying to the said mold a varnish like coating and heating the said mold to a temperature sufficiently high to cause the said coating to blister.

2. The method of preparing metallic molds for casting metal consisting in applying to the said mold a varnish like coating and heating the said mold to a temperature sufficiently high to cause the said coating to blister while the said coating is drying.

3. The method of preparing metallic molds for casting metal consisting in coating the said mold with a varnish like material while the said mold is maintained at a temperature sufficiently high to cause the said applied coating to form blisters.

4. The method of preparing metallic molds for casting metal consisting in coating the said mold with a varnish like material while the said mold is maintained at a temperature sufficiently high to cause the said

applied coating to form blisters and then breaking many of the said blisters.

5. The method of preparing metallic molds for casting metal consisting in coating the said mold with a varnish like material while the said mold is maintained at a temperature sufficiently high to cause the said applied coating to form blisters and then mechanically breaking many of the said blisters.

6. The method of preparing metallic molds for casting metal consisting in coating the said mold with a varnish like material being an admixture comprising evaporated cellulose pulp waste liquor and water while maintaining the said mold at a temperature sufficiently high to cause the said admixture to blister.

7. The method of preparing metallic molds for casting metal consisting in coating the said mold with a varnish like material being an admixture comprising evaporated cellulose pulp waste liquor and water while maintaining the said mold at a temperature of approximately 450° F.

8. The method of preparing metallic molds for casting metal consisting in coating the said mold with a varnish like material being an admixture comprising evaporated cellulose pulp waste liquor and water while maintaining the said mold at a temperature sufficiently high to cause the said applied admixture to blister and then mechanically breaking the said blisters.

9. A metal mold for casting metal having a surface coated with nonmetallic blisters.

10. A metal mold for casting metal having a surface coated with nonmetallic broken blisters.

Signed at Philadelphia, county of Philadelphia, State of Pennsylvania, this 23 day of July, 1930.

FRANK S. CARLILE.